

## UNITED STATES PATENT OFFICE

2,655,428

## METHOD OF WOOL SCOURING WITH COMPOSITION CONTAINING SUINT, ALCOHOLS, KETONES, AND INORGANIC ELECTROLYTES

Harold P. Lundgren, Berkeley, and Willie Fong, San Francisco, Calif., assignors to United States of America as represented by the Secretary of Agriculture

No Drawing. Application March 27, 1950,  
Serial No. 152,271

6 Claims. (Cl. 8—139)

(Granted under Title 35, U. S. Code (1952),  
sec. 266)

1

This application is made under the act of March 3, 1883, as amended by the act of April 30, 1928, and the invention herein described, if patented in any country, may be manufactured and used by or for the Government of the United States of America for governmental purposes throughout the world without any payment to us of any royalty thereon.

This invention relates to the processing of wool and has as its prime object the provision of improved methods for scouring raw wool.

Raw wool scouring is the preliminary step in the processing of wool in which the impurities present in the wool are removed by suitable physical or chemical means. The process is of great importance in the success of subsequent operations, such as carding, drawing, spinning, weaving, dyeing, etc.

The nature and the quantity of the impurities in raw wool vary, depending to a certain extent upon the breed of the animal and the geographical, climatic or nutritional conditions under which it is raised. Generally speaking, these impurities may be classified into two broad categories, (1) acquired impurities, such as earthy material, vegetable matter, faecal matter, paint, tar, etc., and (2) the natural impurities secreted by the animal.

These natural impurities consist of two major components, wool suint and wool grease. Together these two components are commonly known as wool yolk.

Wool suint is the dried, water-soluble material secreted by the sweat gland of the animal. Chemically, very little is known concerning the exact composition of this substance; however, investigators agree that it consists essentially of the potassium salts of high molecular weight fatty acids. Wool suint possesses some detergent power which is utilized in the known aqueous scouring processes as will be explained herein-after.

The wool grease is a complex water-insoluble mixture of fats and oils secreted by the sebaceous glands of the sheep. This material protects the wool fibers against the elements during its growth. Strictly speaking, the greasy component of wool is a wax, the ester of a high molecular weight monohydric alcohol and a fatty acid. The component wool wax alcohols consist of three major series: (1) the sterols, principally cholesterol, (2) the tri-terpene-like alcohols, principally lanosterol, and (3) aliphatic alcohols. The component wool wax acids consist of four major series: (1) the normal fatty acids, (2)

hydroxy acids, (3) branched chain acids, and (4) iso acids.

Commercially, the greater portion of the wool scoured in this country, as well as abroad, is accomplished by aqueous means in an alternating series of bowls and squeeze rolls through which the wool is propelled with a gentle mechanical action. In this aqueous process there are two basic systems known as the emulsification process and the Duhamel or suint process, respectively. In the emulsification process, soap or synthetic detergent and soda ash, added in varying amounts to all bowls except the final rinse bowl, perform the major scouring action. In the suint scouring process, the wool is first steeped in luke-warm water to dissolve the water-soluble suint salts. This suint solution is then clarified by filtering and centrifuging and returned to the first two bowls as the major scouring agent.

Neither the emulsification nor the suint process are entirely satisfactory for the following reasons. In the case of the emulsification process, the pH of the scouring solution is so high that there is danger of serious damage to the wool fibers. Further, the recovery of the by-products, the suint and the wool grease, from the spent scouring liquor is difficult. In the suint process the treatment is mild and does not damage the fibers but it does not reduce the grease content of the wool to the low levels required by the industry.

It has now been found that raw wool can be scoured by a simple and effective method. In essence, our process involves scouring the wool with water containing a neutral, polar, oxygenated organic compound and preferably containing a neutral electrolyte in addition to the organic compound. During the scouring treatment, the suint from the raw wool dissolves in the scouring medium and its effectiveness in emulsifying grease is enhanced by the presence of the afore-mentioned agent or agents. Thus our process is an improvement on the known suint process in that we utilize the emulsification properties of the suint which dissolve in the aqueous scouring medium but we increase the effectiveness of this material. An advantage of the process of this invention is that we preserve the mild action of the suint process and at the same time increase its effectiveness so that the raw wool is scoured to form a finished wool of low grease content as required in commerce.

The scoured wool produced in accordance with our process is not only low in residual grease content but is in a clean and lofty state and

2

relatively free of residual ash. Another feature of our process is the decreased tendency for the fibers to felt during the scouring procedure. Furthermore, our scouring process is performed under mild conditions, at essentially neutral pH, and therefore the wool does not undergo chemical damage or loss in tensile strength or resilience.

In our process, the addition of the neutral, polar, oxygenated organic compound, or organic compound plus neutral electrolyte, to the scouring medium is believed to assist the removal of grease in two ways: (1) By enhancing micelle formation of the suint ions to assist in solubilizing the wool grease; (2) By removal of a protective water shell around the grease particles so that the suint can more effectively remove the grease by solubilization. These factors are further explained as follows:

(1) The chemical structure of the suint salts is similar to that of a typical soap, being characterized by a negatively charged polar or water compatible head and a long chain hydrocarbon or water incompatible tail. The suint salts are readily soluble in water and go into solution as ions. Ordinarily, the suint ions tend to aggregate in water to some extent; the micelles which form consist of the hydrocarbon tails oriented together and the negative heads forming an interface at the water boundary. As many as 20 to 50 ions can be so involved. It is believed that the micelle form of the suint is capable of solubilizing the water-insoluble wool grease in the micelle hydrocarbon core. In the known suint process, the efficiency of scouring is limited in its effect depending upon the degree of micelle formation of the suint salts dissolved in the scouring medium. In our process, the addition of the neutral, polar, oxygenated organic compound or organic compound and electrolyte to the scouring medium, by altering the dielectric constant and ionic strength of the scouring medium, is believed to favor formation of suint micelles. Thus in our process, advantage is taken of factors which further the formation of micelles whereby the capacity of the suint to solubilize wool grease is markedly increased.

(2) In the natural state, the wool grease is hydrated, that is, each particle of the grease is surrounded by a protecting shell of water. This water acts as a barrier to the interaction of the suint salts or micelles and the grease. By adding the neutral, polar, oxygenated organic compound, or organic compound plus neutral electrolyte, to the scouring medium, this barrier is removed by the greater attraction of the aforesaid organic compound, or organic compound plus electrolyte, for water. After removal of this barrier, the grease can be readily solubilized by the suint salts or micelles.

Our invention is thus primarily directed to an improvement in the known suint method of scouring wool wherein the suint derived from the wool is the active scouring agent and the added neutral, polar, oxygenated organic compound, or organic compound plus neutral electrolyte, enhances the effectiveness of the suint as a scouring agent. However, it is not essential to utilize the suint as the sole scouring agent. Thus one may add a soap or a synthetic detergent to the scouring medium. In such case the same effect is obtained as with suint alone, i. e., the scouring action of the added emulsifying agent (soap or synthetic detergent) is enhanced by the presence of the added neutral, polar oxygenated

organic compound, or organic compound plus neutral electrolyte. The point is that the latter agent or agents increase micelle formation of whatever emulsification agent is employed and further act to dehydrate the grease particles, all as described hereinabove. In applying this modification of our invention, one can add to the scouring medium any soap or synthetic detergent commonly used in emulsifying and detergent applications. Thus, one may use any of the well-known alkyl sulphate, alkyl sulphonate, or alkyl aromatic sulphonate detergents. It is known that besides the sulphate or sulphonate group (the hydrophilic group) the compound must also contain a high-molecular weight hydrocarbon or hydrophobic group. There must be a balance between these opposed groups to give the compound the requisite detergent properties. Usually the hydrocarbon group must contain about 8 to 18 carbon atoms in the case of alkyl sulphates or sulphonates and about 14 to 28 carbon atoms in the case of alkyl aromatic sulphonates to give the proper balance. These compounds are generally employed in the form of their salts, i. e., their potassium, sodium, ammonium, or amine salts. Some of the particular detergents which we may use are: sodium octyl sulphate, sodium nonyl sulphate, sodium decyl sulphate, sodium undecyl sulphate, sodium dodecyl sulphate, sodium tridecyl sulphate, sodium tetradecyl sulphate, sodium pentadecyl sulphate, sodium hexadecyl sulphate, sodium heptadecyl sulphate, sodium octadecyl sulphate, sodium oleyl sulphate, sodium octyl sulphonate, sodium nonyl sulphonate, sodium decyl sulphonate, sodium undecyl sulphonate, sodium dodecyl sulphonate, sodium tridecyl sulphonate, sodium tetradecyl sulphonate, sodium pentadecyl sulphonate, sodium hexadecyl sulphonate, sodium octadecyl sulphonate, sodium oleyl sulphonate, sodium salt of di-octyl sulphosuccinate, sodium octyl benzene sulphonate, sodium nonyl benzene sulphonate, sodium decyl benzene sulphonate, sodium undecyl benzene sulphonate, sodium dodecyl benzene sulphonate, sodium tridecyl benzene sulphonate, sodium tetradecyl benzene sulphonate, sodium pentadecyl benzene sulphonate, sodium hexadecyl benzene sulphonate, sodium heptadecyl benzene sulphonate, sodium octadecyl benzene sulphonate, sodium tri(isopropyl) benzene sulphonate, sodium tri(isobutyl) benzene sulphonate, sodium tri(isopropyl) naphthalene sulphonate, sodium tri(isobutyl) naphthalene sulphonate, and so forth. The commercially-available detergents are generally not pure compounds but are mixtures of homologous compounds and are quite satisfactory. Thus, for example, the sodium alkyl benzene sulphonate wherein the alkyl group contains 12 to 18 carbon atoms is a well known detergent. Others are: a mixture of sodium alkyl sulphates consisting mostly of sodium lauryl sulphate; a mixture of sodium alkyl phenol sulphonates wherein the alkyl group contains 12 to 18 carbon atoms; and a mixture of sodium alkyl sulphonates wherein the alkyl group contains 10 to 18 carbon atoms. It is evident that the particular detergent used is not critical except that one should be chosen which is generally useful in emulsifying and detergent applications. Regardless of the type of compound chosen, its efficiency to scour wool will be enhanced by applying the teachings of this invention.

Many different agents within the class of

neutral, polar, oxygenated organic compounds can be used in our process. Aliphatic alcohols having 1 to 8 carbon atoms, tetrahydrofurfuryl alcohol, and aliphatic ketones having 3 to 6 carbon atoms are included. The following are examples of suitable aliphatic alcohols and ketones in this category: methanol, ethanol, normal propanol, isopropanol, normal butanol, tertiary butanol, butanol-2, isobutanol (2-methyl-propanol-1), amyl alcohols, hexyl alcohols, heptyl alcohols, octyl alcohols, ethylene glycol, propylene glycol, glycerol, ethylene glycol monomethyl ether, ethylene glycol monomethyl ether, acetone, diacetone alcohol, methyl ethyl ketone, and so forth. If desired, mixtures can be used instead of individual compounds. Thus for example the commercially-available ethanol denatured with methanol is suitable.

In general, the concentration of the neutral, polar, oxygenated organic compound may be varied from about 0.1% to about 50%. The particular concentration to use in any specific situation depends on many factors as, for example, the nature of the raw wool and especially the nature of the grease and suint associated therewith, the temperature of scouring, the concentration of electrolytes in the scouring solution, the micelle-forming potency of the particular organic compound used, the mechanical efficiency of the scouring process as for instance the degree of agitation, number of scouring operations, efficiency of rinsing, and so forth. The concentration required in any particular case can be easily determined by scouring small samples of wool using varying concentrations of the organic solvent and noting which concentration gives the lowest residual grease content in the scoured wool. Under the conditions used in the experiments set forth in the examples we have found that the following concentrations give good results with some particular compounds:

| Compound                               | Concentration range giving substantial increase in scouring efficiency, percent | Approx. concentration giving maximum scouring efficiency, percent |
|----------------------------------------|---------------------------------------------------------------------------------|-------------------------------------------------------------------|
| Methanol                               | 10-50                                                                           | 40                                                                |
| Ethanol                                | 5-40                                                                            | 20                                                                |
| n-Propanol                             | 5-30                                                                            | 20                                                                |
| Isopropanol                            | 5-25                                                                            | 10                                                                |
| n-Butanol                              | 1-6                                                                             | 3                                                                 |
| n-Pentanol                             | 0.5-3                                                                           | 2.5                                                               |
| n-Hexanol                              | 0.1-0.6                                                                         | .5                                                                |
| Acetone                                | 5-40                                                                            | 25                                                                |
| Methanol in presence of electrolyte    | 5-40                                                                            | 30                                                                |
| Ethanol in presence of electrolyte     | 5-40                                                                            | 20                                                                |
| n-Propanol in presence of electrolyte  | 5-25                                                                            | 10                                                                |
| Isopropanol in presence of electrolyte | 5-15                                                                            | 10                                                                |
| n-Butanol in presence of electrolyte   | 0.5-6                                                                           | 3                                                                 |
| n-Pentanol in presence of electrolyte  | 0.25-2.5                                                                        | 1                                                                 |
| n-Hexanol in presence of electrolyte   | 0.1-0.6                                                                         | .4                                                                |
| Acetone in presence of electrolyte     | 5-40                                                                            | 20                                                                |

With regard to the electrolyte, one may use many different salts, since the critical point is to supply inorganic ion to the scouring solution. Thus one can use any neutral, soluble salt of the alkali metals such as sodium, potassium or of ammonium. Suitable salts are, for example, alkali metal or ammonium chlorides, sulphates, nitrates, bromides, iodides, fluorides, and so forth. The electrolyte is generally employed in a concentration from about 0.05 to about 0.5 normal. In most instances a concentration of about 0.1 normal is preferred. Salts of magnesium, calcium or other metals which cause precipitation of insoluble suint salts cannot be

course be used in the electrolyte. For the same reason the water used for scouring should be essentially free from calcium, magnesium, iron and similar metals, that is, the water should be soft. If only hard water is available, it is evident that a small amount of calcium-sequestering agent may be added to counteract the hardness. Suitable agents are, for example, alkali metal hexametaphosphates, citrates, pyrophosphates, etc.

The scouring treatment is generally effected at temperatures customarily used in scouring wool by the known emulsification or suint procedures, i. e., from about 20° C. to about 70° C. Preferably, our procedure is carried out at an elevated temperature, namely, from about 40° C. to about 60° C. to facilitate emulsification of the wool grease.

The following examples exhibit the invention in greater detail. It is understood that these examples are furnished only by way of illustration and not limitation.

For use in the experiments set forth in the examples, a standard raw wool was prepared as follows: A lot of raw California wool of medium fineness was opened and blended five times in an experimental type opener. The opened wool was then homogenized by repeated hand carding and mixing. This standard wool had a shrinkage of approximately 40% and a grease content of 12% as determined by solvent extraction. The scouring tests were performed by a standardized technique with provisions for uniform control of temperature and the degree of mechanical agitation.

#### Example I

An aqueous solution was prepared containing 2% normal butanol and sodium chloride in a concentration of 0.1 normal.

Four hundred ml. of this solution was placed in a beaker and 3 grams of raw wool was agitated in the solution for 3 minutes while maintaining the temperature at 60° C. The washed wool was squeezed free of solution and re-washed in 400 ml. of a fresh batch of the solution again agitating for 3 minutes at 60° C. The wool was then squeezed free of solution, washed with water, dried and the grease content determined by Soxhlet extraction with benzene. The residual grease content was found to be 0.5%.

The scouring procedure as set forth above was repeated using different scouring solutions, i. e., (a) water, alone; (b) water containing varying concentrations of n-butanol; and (c) water containing sodium chloride in a concentration of 0.1 normal and varying concentrations of n-butanol. The results obtained in these experiments and those obtained from the experiment above are tabulated below:

TABLE I

| Expt. No.   | Scouring solution            | Residual grease content of wool, percent |
|-------------|------------------------------|------------------------------------------|
| 1 (control) | water                        | 8.7                                      |
| 2           | 1% n-butanol                 | 6.46                                     |
| 3           | 2% n-butanol                 | 3.06                                     |
| 4           | 3% n-butanol                 | .85                                      |
| 5           | 4% n-butanol                 | 1.22                                     |
| 6           | 5% n-butanol                 | 2.52                                     |
| 7           | 6% n-butanol                 | 6.99                                     |
| 8           | 1% n-butanol plus 0.1 N NaCl | .85                                      |
| 9           | 2% n-butanol plus 0.1 N NaCl | .50                                      |
| 10          | 3% n-butanol plus 0.1 N NaCl | .74                                      |
| 11          | 4% n-butanol plus 0.1 N NaCl | .67                                      |
| 12          | 5% n-butanol plus 0.1 N NaCl | 1.48                                     |

7  
Example II

The scouring procedure of Example I was repeated using as the scouring solution aqueous solutions of methanol and aqueous solutions of methanol containing sodium chloride in a concentration of 0.1 normal. The following results were obtained:

TABLE 2

| Expt. No. | Scouring solution            | Residual grease in wool, percent |
|-----------|------------------------------|----------------------------------|
| 1.        | 10% methanol                 | 6.97                             |
| 2.        | 20% methanol                 | 4.67                             |
| 3.        | 30% methanol                 | 3.32                             |
| 4.        | 40% methanol                 | 2.78                             |
| 5.        | 50% methanol                 | 5.42                             |
| 6.        | 10% methanol plus 0.1 N NaCl | 3.84                             |
| 7.        | 20% methanol plus 0.1 N NaCl | 1.97                             |
| 8.        | 30% methanol plus 0.1 N NaCl | 1.12                             |
| 9.        | 40% methanol plus 0.1 N NaCl | 3.81                             |
| 10.       | 50% methanol plus 0.1 N NaCl | 7.19                             |

## Example III

The scouring procedure as set forth in Example I was repeated using as the scouring solution aqueous solutions of ethanol and aqueous solutions of ethanol containing sodium chloride in varying concentrations. The following results were obtained:

TABLE 3

| Expt. No. | Scouring solution           | Residual grease in wool, percent |
|-----------|-----------------------------|----------------------------------|
| 1.        | 10% ethanol                 | 2.26                             |
| 2.        | 20% ethanol                 | 1.32                             |
| 3.        | 30% ethanol                 | 2.28                             |
| 4.        | 10% ethanol plus 0.1 N NaCl | .89                              |
| 5.        | 10% ethanol plus 0.2 N NaCl | .81                              |
| 6.        | 10% ethanol plus 0.3 N NaCl | .93                              |
| 7.        | 10% ethanol plus 0.4 N NaCl | 1.84                             |
| 8.        | 20% ethanol plus 0.1 N NaCl | .70                              |
| 9.        | 30% ethanol plus 0.1 N NaCl | 2.14                             |

## Example IV

The scouring procedure as set forth in Example I was repeated using as the scouring solution aqueous solutions of normal propanol and isopropanol. The following results were obtained:

TABLE 4

| Expt. No. | Scouring solution               | Residual grease content of wool, percent |
|-----------|---------------------------------|------------------------------------------|
| 1.        | 10% n-propanol plus 0.1 N NaCl  | 0.81                                     |
| 2.        | 20% n-propanol plus 0.1 N NaCl  | 3.08                                     |
| 3.        | 10% isopropanol                 | 1.37                                     |
| 4.        | 10% isopropanol plus 0.1 N NaCl | .98                                      |
| 5.        | 20% isopropanol plus 0.1 N NaCl | 1.91                                     |

## Example V

The scouring procedure as set forth in Example I was repeated using as the scouring solution aqueous solutions of normal amyl alcohol and aqueous solutions of normal amyl alcohol containing sodium chloride. The following results were obtained:

8  
TABLE 5

| Expt. No. | Scouring solution                   | Residual grease content of wool, percent |
|-----------|-------------------------------------|------------------------------------------|
| 1.        | 0.5% n-amyl alcohol                 | 6.09                                     |
| 2.        | 1% n-amyl alcohol                   | 3.87                                     |
| 3.        | 1.5% n-amyl alcohol                 | 2.53                                     |
| 4.        | 2% n-amyl alcohol                   | 2.19                                     |
| 5.        | 2.5% n-amyl alcohol                 | 1.69                                     |
| 6.        | 0.5% n-amyl alcohol plus 0.1 N NaCl | 1.62                                     |
| 7.        | 1% n-amyl alcohol plus 0.1 N NaCl   | .72                                      |
| 8.        | 1.5% n-amyl alcohol plus 0.1 N NaCl | 1.23                                     |
| 9.        | 2% n-amyl alcohol plus 0.1 N NaCl   | 3.54                                     |
| 10.       | 2.5% n-amyl alcohol plus 0.1 N NaCl | 3.10                                     |

## Example VI

The scouring procedure as set forth in Example I was repeated using as the scouring solution aqueous solutions of normal hexanol and aqueous solutions of this alcohol containing sodium chloride. The following results were obtained:

TABLE 6

| Expt. No. | Scouring solution              | Residual grease content of wool, percent |
|-----------|--------------------------------|------------------------------------------|
| 1.        | 0.1% n-hexanol                 | 6.00                                     |
| 2.        | 0.2% n-hexanol                 | 5.91                                     |
| 3.        | 0.3% n-hexanol                 | 5.09                                     |
| 4.        | 0.4% n-hexanol                 | 4.96                                     |
| 5.        | 0.5% n-hexanol                 | 3.63                                     |
| 6.        | 0.6% n-hexanol                 | 4.90                                     |
| 7.        | 0.1% n-hexanol plus 0.1 N NaCl | 4.45                                     |
| 8.        | 0.2% n-hexanol plus 0.1 N NaCl | 3.27                                     |
| 9.        | 0.3% n-hexanol plus 0.1 N NaCl | 1.55                                     |
| 10.       | 0.4% n-hexanol plus 0.1 N NaCl | .62                                      |
| 11.       | 0.5% n-hexanol plus 0.1 N NaCl | .72                                      |
| 12.       | 0.6% n-hexanol plus 0.1 N NaCl | .74                                      |

## Example VII

The scouring procedure as set forth in Example I was repeated using as the scouring solution aqueous solutions of acetone and aqueous solutions of acetone containing sodium chloride. The following results were obtained:

TABLE 7

| Expt. No. | Scouring solution           | Residual grease content of wool, percent |
|-----------|-----------------------------|------------------------------------------|
| 1.        | 10% acetone                 | 4.53                                     |
| 2.        | 20% acetone                 | 1.95                                     |
| 3.        | 30% acetone                 | 2.17                                     |
| 4.        | 40% acetone                 | 5.08                                     |
| 5.        | 10% acetone plus 0.1 N NaCl | 2.21                                     |
| 6.        | 20% acetone plus 0.1 N NaCl | .88                                      |
| 7.        | 30% acetone plus 0.1 N NaCl | 3.28                                     |
| 8.        | 40% acetone plus 0.1 N NaCl | 7.17                                     |

Having thus described our invention, we claim:

1. In the process of scouring raw wool with an essentially-neutral aqueous medium wherein the active scouring agent is suint derived from raw wool, the improvement which comprises incorporating with the aqueous medium a neutral, polar, oxygenated organic compound selected from the group consisting of aliphatic alcohols having 1 to 8 carbon atoms, tetrahydrofurfuryl alcohol, and aliphatic ketones having 3 to 6 carbon atoms in a concentration from about 0.1% to about 50%, and a neutral, inorganic electrolyte selected from the group consisting of the water-soluble salts of the alkali metals and ammonium in a concentration from about 0.05 to about 0.5 normal.

9

2. The process of claim 1 wherein the neutral, polar, oxygenated organic compound is isopropanol in a concentration about from 5 to 15%.

3. The process of claim 1 wherein the neutral, polar, oxygenated organic compound is n-propanol in a concentration about from 5 to 25%.

4. The process of claim 1 wherein the neutral, polar, oxygenated organic compound is n-butanol in a concentration about from 0.5 to 6%.

5. The process of claim 1 wherein the neutral, polar, oxygenated organic compound is n-amyl alcohol in a concentration about from 0.25 to 2.5%.

6. The process of claim 1 wherein the neutral, polar, oxygenated organic compound is ethanol in a concentration about from 5 to 40%.

HAROLD P. LUNDGREN.  
WILLIE FONG.

## References Cited in the file of this patent

20

## UNITED STATES PATENTS

| Number | Name    | Date          |
|--------|---------|---------------|
| 13,206 | Barrows | July 10, 1855 |

10

| Number       | Name           | Date          |
|--------------|----------------|---------------|
| 163,729      | Braun          | May 25, 1875  |
| 1,377,790    | Poole          | May 10, 1921  |
| 1,717,439    | Duhamel        | June 18, 1929 |
| 5 1,717,440  | Duhamel        | June 18, 1929 |
| 1,987,583    | Berthold       | Jan. 8, 1935  |
| 2,097,737    | Pickett et al. | Nov. 2, 1937  |
| 2,221,933    | Eitelman       | Nov. 19, 1940 |
| 2,283,421    | Castendyk      | May 19, 1942  |
| 10 2,404,913 | Leiserson      | July 30, 1946 |

## FOREIGN PATENTS

| Number    | Country       | Date          |
|-----------|---------------|---------------|
| 1,123     | Great Britain | 1870          |
| 15 25,321 | Great Britain | 1909          |
| 308,605   | Great Britain | June 23, 1930 |
| 352,989   | Great Britain | July 9, 1931  |
| 586,540   | Great Britain | Mar. 21, 1947 |

## OTHER REFERENCES

Thompson, "Practice and Theory in Scouring of Raw Wool—II." The Textile Manufacturer, January 1937, pages 5, 6, 8-139.